

# United States Patent Office

2,761,778

Patented Sept. 4, 1956

1

2,761,778

## ALLOY

Herman L. Mann, New York, N. Y.

No Drawing. Application August 26, 1953,  
Serial No. 376,759

4 Claims. (Cl. 75—171)

1

2

## Example 2

| Metal:    | Per cent by weight |
|-----------|--------------------|
| Chromium  | 12 to 18           |
| Cobalt    | 5 to 20            |
| Nickel    | 45 to 60           |
| Copper    | 18 to 26           |
| Beryllium | .25 to 1.0         |

| Metal:    | Per cent by weight |
|-----------|--------------------|
| Chromium  | 15                 |
| Cobalt    | 5                  |
| Nickel    | 54                 |
| Copper    | 25                 |
| Beryllium | 1                  |

## Example 3

| Metal:    | Per cent by weight |
|-----------|--------------------|
| Chromium  | 15                 |
| Cobalt    | 5                  |
| Nickel    | 54                 |
| Copper    | 25                 |
| Beryllium | 1                  |

These alloys have a melting point between 2300° and 2500° F. They can be cast in a gypsum refractory to produce a satisfactory denture.

Among the advantages of this alloy in the manufacture of dentures is the light color of the alloy. Another advantage is the smooth surface of the product cast with this alloy which minimizes the amount and expense of finishing by polishing. As the alloy of this invention is resistant to acid including nitric acid, a denture formed of this alloy resists mouth acids. As this alloy has a low atomic weight the cubic volume occupied by this alloy is greater per unit of weight and the denture is correspondingly less expensive.

The beryllium which may be used in the alloy of this invention serves as a de-oxidizer to remove impurities and may be considered a scavenger in its function in the alloy of this invention.

The copper employed in the alloy of this invention acts to lower the fusing point and gives better flow properties to the alloy in casting and produces a product with a smoother surface.

Various changes may be made in the above described embodiments of this invention without departing from the spirit of the invention which is limited only by the appended claims.

I claim:

1. An alloy having as its principal ingredients chromium, nickel, cobalt and copper and containing chromium from 12 to 18 per cent by weight, cobalt from 5 to 20 per cent by weight, nickel from 45 to 60 per cent by weight, copper from 18 to 26 per cent by weight and beryllium from .25 to 1.0 per cent by weight.

2. An alloy consisting of chromium, nickel, cobalt and copper, the chromium content being 12% to 18% by weight, the nickel content being 45% to 60% by weight, the cobalt content being 5% to 20% by weight and the copper content being 18% to 26% by weight, said alloy being characterized by a low fusing point and resistance to acids.

3. An alloy consisting of chromium, nickel, cobalt, copper and beryllium and containing, by weight, 12% to 18% chromium, 5% to 20% cobalt, 45% to 60% nickel, 18% to 26% copper and .25% to 1.0% beryllium.

4. A denture formed from an alloy consisting of by weight, 15% chromium, 5% cobalt, 54% nickel, 25% copper and 1% beryllium.

## References Cited in the file of this patent

### UNITED STATES PATENTS

|           |         |               |
|-----------|---------|---------------|
| 2,521,273 | Wissler | Sept. 5, 1950 |
| 2,636,818 | Low     | Apr. 28, 1953 |

### FOREIGN PATENTS

|         |               |              |
|---------|---------------|--------------|
| 485,226 | Great Britain | May 17, 1938 |
|---------|---------------|--------------|

## Example 1

| Metal:   | Per cent by weight |
|----------|--------------------|
| Chromium | 12 to 18           |
| Cobalt   | 5 to 20            |
| Nickel   | 45 to 60           |
| Copper   | 18 to 26           |